

W. D. COOLIDGE,  
METHOD OF MAKING INCANDESCENT LAMPS,  
APPLICATION FILED NOV. 7, 1910.

1,230,869.

Patented June 26, 1917.



Witnesses:

Earl G. Klock.  
J. Elbi Eler

Inventor:

William D. Coolidge,  
by Almon D. Dens  
His Attorney.

# UNITED STATES PATENT OFFICE.

WILLIAM D. COOLIDGE, OF SCHENECTADY, NEW YORK, ASSIGNOR TO GENERAL ELECTRIC COMPANY, A CORPORATION OF NEW YORK.

## METHOD OF MAKING INCANDESCENT LAMPS.

1,230,869.

Specification of Letters Patent. Patented June 26, 1917.

Original application filed June 14, 1907, Serial No. 378,936. Divided and this application filed November 7, 1910. Serial No. 591,187.

*To all whom it may concern:*

Be it known that I, WILLIAM D. COOLIDGE, a citizen of the United States, residing at Schenectady, county of Schenectady, State of New York, have invented certain new and useful Improvements in Methods of Making Incandescent Lamps, (division of my application filed June 14, 1907, Serial No. 378,936,) of which the following is a specification.

My present invention has for its object a method of assembling tungsten lamps which consists in winding the tungsten filament on a spider, similar, for instance, to those used in tantalum lamps, while the tungsten filament is in a heated and pliant condition.

The scope of my invention is pointed out in the appended claims, for a better understanding of which reference may be had to the following detailed description taken in connection with the accompanying drawings, in which the figure is a perspective view of a lamp made according to the procedure herein disclosed.

Tungsten powder of relatively good quality can be readily produced by reduction of tungsten tri-oxid with hydrogen according to well-known chemical methods. The powder so obtained is non-coherent and exceedingly refractory but can be shaped into coherent conductors suitable for the practice of my present invention. Several methods of constructing such coherent conductors are known in the art but the one preferred by me in the practice of my present invention is here described in some detail. It is not claimed by me in this application as it forms the subject-matter of my application, Serial No. 377,781, filed June 7, 1907, issued as Patent No. 1,026,343, May 14, 1912. This preferred method of making coherent conductors is as follows:

The tungsten powder is rubbed into a warm and plastic amalgam, consisting of say equal parts of cadmium and mercury, forming a homogeneous ductile mixture; the tungsten may be added in the proportion of 30 per cent. or more by weight of the final mixture. This mixing operation may be carried out in an ordinary chemist's mortar by rubbing the materials with a pestle.

The product thus obtained may be squirted warm through a diamond die and may be otherwise manipulated without difficulty.

The squirted wires probably consist of a mere mechanical mixture of the tungsten powder with the amalgam. The proportion of mercury and cadmium in the amalgam may be varied through relatively wide limits and a very suitable mixture consists of 44 parts cadmium to 56 parts mercury. Other binders can be used in place of the cadmium amalgam, as for instance cadmium-bismuth alloy having 112 parts cadmium to 208 parts bismuth; or an alloy containing mercury-cadmium and bismuth in the following proportions: mercury 53 parts, cadmium 42 parts and bismuth 5 parts. It will be noted that all the materials of the binder have relatively low vaporization points and can therefore be distilled at low temperatures.

To remove the vaporizable components above mentioned, I may bake the wires in an evacuated tube to the temperature at which most of the mercury and part of the cadmium vaporize out; this leaves a relatively strong and somewhat brittle residue, consisting mainly of tungsten and cadmium, and also bismuth, if the latter has been used in the binder. The wires may then be removed from the baking receptacle and suspended between conductive metal clips or terminals in a treating bulb or tube and there subjected to the heating action of current passed through the wires. A vacuum or inert atmosphere should be maintained about the wires during this treatment. The current distils or vaporizes the remaining cadmium or other component of the binding material and then consolidates the porous residue of tungsten into a homogeneous and relatively compact wire. The tungsten particles seem to sinter together and thus decrease the porosity of the structure. The wire shrinks in length very materially during treatment. The wire is then allowed to cool and when taken from the treating chamber is found to be strong and firm and somewhat elastic but without the capability of taking a permanent set and practically devoid of ductility, at least in the sense in which that term is applied to such metals as copper, silver, platinum, etc.

To construct a tungsten lamp from a coherent conductor produced as above described or in any other suitable manner, I proceed by winding the conductor on a spider or

supporting frame, similar, for instance, to those used in tantalum lamps, while maintaining the tungsten in a pliant condition by the application of heat. The tungsten conductor may be heated by the continuous passage of current through it or in any other suitable way. I may even secure the desired mobility by merely heating the ends of the supporting spider while the filament is being bent around them. As soon as the tungsten is heated sufficiently it becomes soft and feels pliant like copper wire. All these manipulations can be carried out while the tungsten is at a temperature somewhat above room temperature, but lower than visible redness and lower than the temperature at which tungsten appears to oxidize in air. The manipulations can, therefore, be conducted in open air.

20 The finished product may take the form shown in the drawing wherein the bent tungsten filament 1 is shown mounted on a supporting structure 2 of a type commonly used in tantalum lamps.

25 What I claim as new and desire to secure by Letters Patent of the United States is:

1. The process of mounting a continuous brittle tungsten filament on the supports of an incandescent lamp which consists in rendering said filament pliant by heating it while exposed to the atmosphere to a temperature below that at which appreciable oxidation takes place and below that corre-

sponding to visible redness, and winding the filament on said supports while at said temperature.

2. The process of mounting a continuous brittle tungsten filament on the supports of an incandescent lamp which consists in heating the portions to be bent while exposed to the atmosphere to a temperature that renders them pliable and is below that of appreciable oxidation and below that corresponding to visible redness of the filament, and stringing the filament on said supports in the open air while said filament and said supports are exposed to permit manipulation of the filament.

3. The process of mounting a continuous sintered tungsten filament in zigzag form on the supports of an incandescent lamp which consists in rendering the filament pliant by passing current through it to heat it while exposed to the atmosphere to a temperature below that which corresponds to visible redness of the filament and below that at which appreciable oxidation takes place, and stringing said filament while still hot and pliant on said supports with said filament and said supports in the open air.

In witness whereof, I have hereunto set my hand this 4th day of November, 1910.

WILLIAM D. COOLIDGE.

Witnesses:

BENJAMIN B. HULL,  
HELEN ORFORD.